# EUROPEAN PATENT APPLICATION

(11) **EP 3 719 162 A1**
(43) Date of publication of application: **07.10.2020**
(21) Application number: 18883591.2
(22) Date of filing: 27.07.2018
(51) Int. Cl.: C22C 38/44, C22C 38/46, C22C 38/50, C22C 38/48, C22C 38/58, C21D 8/02, C21D 9/46

(54) **HIGH STRENGTH STEEL MATERIAL HAVING EXCELLENT HYDROGEN-INDUCED CRACKING RESISTANCE AND LOW-TEMPERATURE IMPACT TOUGHNESS AND MANUFACTURING METHOD THEREFOR**

(30) Priority: 01.12.2017 KR 20170164465
(71) Applicant: POSCO, Nam-gu Pohang-si, Gyeongsangbuk-do 37859 (KR)
(72) Inventor: UM, Kyung-Keun, Pohang-si Gyeongsangbuk-do 37877 (KR); KIM, Dae-Woo, Pohang-si Gyeongsangbuk-do 37877 (KR)
(74) Representative: Potter Clarkson
(86) International application number: PCT/KR2018/008579
(87) International publication number: WO 2019/107700

(57) **Abstract**

The present invention provides a high strength steel material having excellent hydrogen-induced cracking resistance and low-temperature impact toughness and a manufacturing method therefor, the steel material comprising, by weight%, 0.02-0.12% of C, 0.02-0.60% of Si, 0.6-1.6% of Mn, 0.020% or less of P (0% exclusive), 0.003% or less of S (0% exclusive), 0.002-0.060% of Sol.Al, 0.005-0.6% of Cu, 0.005-1.0% of Ni, 0.005-0.5% of Cr, 0.01-0.3% of Mo, 0.001-0.10% of Ti, 0.001-0.06% of Nb, 0.001-0.10% of V, 0.001-0.006% of N, 0.0002-0.0060% of Ca, and the balance of Fe and inevitable impurities, with (Ti+V+0.5Nb+0.5Mo) being 0.05% or more and (Ti+V+0.5Nb+0.5Mo)/C being 0.8 or greater, the steel material having a microstructure inclusive of ferrite; and at least one of pearlite, cementite, and MA (martensite-austenite complex phase) wherein the ferrite has a fraction of 90% by area or more (100% exclusive) and the at least one of ferrite, cementite, and MA (martensite-austenite complex phase) has a fraction of 10% by area or less and wherein the ferrite structure includes 0.03% by weight or more of fine carbonitride precipitates having an average size of 100 nm or less and is 20 µm or less in average grain size.

## Description

### [Technical Field]

The present disclosure relates to a high-strength steel material used in plant equipment for extracting, processing, transporting, and storing crude oil and shipbuilding and offshore structures, and a method for manufacturing the same, and more specifically, to a high-strength steel material having excellent hydrogen-induced cracking resistance (HIC resistance) and low-temperature impact toughness, and a method for manufacturing the same.

### [Background Art]

Due to depletion of oil resources and high oil prices, production of low-quality crude oil with high contents of impurities, such as sulfur, is gradually increasing. Accordingly, steel materials used in all plant equipment for extracting, processing, transporting, and storing the low-grade crude oil are also required to have properties of inhibiting hydrogen-induced cracking (HIC) caused by wet hydrogen sulfide due to a sulfur component in the crude oil.

In addition, environmental pollution caused by recent safety accidents has become a global issue, and an astronomical cost is required to recover the same. Accordingly, a level of required characteristics of steel materials used in the energy industry is gradually increasing.

As an example of materials of the plant equipment for extracting, processing, transporting, and storing crude oil and shipbuilding and offshore structures, a high-strength normalized steel material has been suggested.

As a method for obtaining high strength for a normalized steel material, an increase in a pearlite fraction by adding C, an addition of a solid solution strengthening element such as Cu and Mo, and production of carbonitride precipitates by simply adding Nb and V have been used.

Meanwhile, as a method for improving HIC resistance of a steel material, controlling internal defects, such as inclusions, voids, or the like, in the steel material, which may cause hydrogen accumulation and cracking, applying strong rolling to minimize hardened structures, such as pearlite, or the like, in which cracking easily occurs and is propagated, or to control a shape thereof, and the like, have been widely proposed and used.

As a demand for higher strength of the steel material gradually increases, however, an amount of C addition or solid solution strengthening component added to increase strength is increasing. An increase in the amount of C addition serves to increase a pearlite fraction and allow the pearlite to have a banded structure, thereby facilitating propagation of HIC and significantly reducing low-temperature impact toughness, which is contradictory.

In addition, an addition of a solid solution strengthening component, such as copper (Cu), nickel (Ni), molybdenum (Mo), or the like, has an effect of increasing strength but may cause surface cracking due to red shortness or cause significantly decrease in economic efficiency due to the high cost thereof.

Further, when excessive amounts of Nb and V are added in order to obtain a strengthening effect by precipitates, hardenability of a weld zone is greatly increased to a higher level than a reference level, causing deteriorated toughness of the weld zone and HIC.

As described above, the conventional method has a problem in that it is difficult to simultaneously secure high strength of normalizing steel material, excellent low-temperature impact toughness and HIC resistance properties.

Accordingly, there is a need to develop a normalizing steel material having high strength, excellent low-temperature impact toughness and HIC resistance properties.

### [Disclosure]

### [Technical Problem]

A preferable aspect of the present disclosure is to provide a high-strength steel material having excellent hydrogen-induced cracking resistance (HIC resistance) and low-temperature impact toughness.

Another preferable aspect is to provide a manufacturing method for the high-strength steel material having excellent hydrogen-induced cracking resistance (HIC resistance) and low-temperature impact toughness.

### [Technical Solution]

According to a preferable aspect of the present disclosure, a high-strength steel material having excellent hydrogen-induced cracking resistance and low-temperature impact toughness, containing, by weight%, 0.02% to 0.12% of carbon (C), 0.02% to 0.60% of silicon (Si), 0.6 to 1.6% of manganese (Mn), 0.02% or less of phosphorus (P) (excluding 0%), 0.003% or less of sulfur (S) (excluding 0%), 0.002% to 0.060% of sol. aluminum (sol.Al), 0.005% to 0.6% of copper (Cu), 0.005% to 1.0% of nickel (Ni), 0.005% to 0.5% of chromium (Cr), 0.01% to 0.3% of molybdenum (Mo), 0.001% to 0.10% of titanium (Ti), 0.001% to 0.06% of niobium (Nb), 0.001% to 0.10% of vanadium (V), 0.001% to 0.006% of nitrogen (N), 0.0002% to 0.0060% of calcium (Ca), a remainder of iron (Fe) and inevitable impurities, with (Ti+V+0.5Nb+0.5Mo) being 0.05% or greater and (Ti+V+0.5Nb+0.5Mo)/C being 0.8 or greater, the steel material having a microstructure inclusive of ferrite; and at least one of pearlite, cementite, and martensite-austenite complex phase (MA), wherein the ferrite has a fraction of 90% by area or more (excluding 100%), and at least one of pearlite, cementite, and martensite-austenite complex phase MA has a fraction of 10% by area or less, and wherein the ferrite includes 0.03 wt% or more of fine carbonitride precipitates having an average size of 100 nm or less and is 20 µm or less in average grain size is provided.

According to an another preferable aspect, a method for manufacturing a high-strength steel material having excellent hydrogen-induced cracking resistance and low-temperature impact toughness, including reheating a slab comprising by weight%, 0.02% to 0.12% of carbon (C), 0.02% to 0.60% of silicon (Si), 0.6 to 1.6% of manganese (Mn), 0.02% or less of phosphorus (P) (excluding 0%), 0.003% or less of sulfur (S) (excluding 0%), 0.002% to 0.060% of sol. aluminum (sol.Al), 0.005% to 0.6% of copper (Cu), 0.005% to 1.0% of nickel (Ni), 0.005% to 0.5% of chromium (Cr), 0.01% to 0.3% of molybdenum (Mo), 0.001% to 0.10% of titanium (Ti), 0.001% to 0.06% of niobium (Nb), 0.001% to 0.10% of vanadium (V), 0.001% to 0.006% of nitrogen (N), 0.0002% to 0.0060% of calcium (Ca), a remainder of iron (Fe) and inevitable impurities, with (Ti+V+0.5Nb+0.5Mo) being 0.05% or greater and (Ti+V+0.5Nb+0.5Mo)/C being 0.8 or greater to 1080°C to 1300°C; hot rolling the reheated slab to a finish hot rolling temperature of 850°C or higher to obtain a hot rolled steel plate; water cooling the hot rolled steel plate to 550°C to 750°C; and performing normalizing heat treatment the cooled steel plate to 850°C to 950°C for 1.3*t [where t refers to thickness of steel plate (mm)] + (5 minutes to 60 minutes) is provided.

The method may further include performing tempering heat treatment the normalizing heat treated steel material to 500°C or higher for 10 minutes or more.

### [Advantageous Effects]

According to a preferable aspect of the present disclosure, a high-strength steel material, which may be effectively applied to plant equipment for extracting, processing, transporting, and storing crude oil, shipbuilding and offshore structures, pressure vessels, and the like, may be provided.

### [Brief Description of Drawings]

FIG. 1 is a photograph of a microstructure of a steel material (Comparative Example 3) manufactured according to a conventional method.
FIG. 2 is a photograph of a microstructure of a steel material (Inventive Example 1) manufactured according to the present disclosure.
FIG. 3 is a photograph illustrating a distribution of a precipitate of the steel material (Comparative Example 3) manufactured according to a conventional method.
FIG. 4 is a photograph illustrating a distribution of a precipitate of the steel material (Inventive Example 1) manufactured according to the present disclosure.

### [Best Mode for Invention]

Hereinafter, preferred embodiments are described.

However, the preferred embodiments of the present disclosure are provided to completely describe so that this disclosure will be thorough and complete, and will fully convey the scope of the disclosure to those skilled in the art.

In addition, the present disclosure may be embodied in many different forms and should not be construed as being limited to the embodiments set forth herein.

As used herein, the term "comprise" and variations such as "comprises" or "comprising," as well as the term "include" and variations such as "includes" and "including," will be understood to imply the inclusion of stated elements but not the exclusion of any other elements.

One of the major ideas of the present disclosure is to provide a microstructure maximally inclusive of a ferrite fraction and minimally inclusive of cementite having a disadvantageous microstructure, and a hard phase such as pearlite, martensite-austenite complex phase (MA), or the like such that HIC propagation resistance and strength are simultaneously secured. To this end, hot rolling (controlled rolling) and water cooling (controlled cooling) are performed to produce nano-sized fine precipitates are produced in ferrite grains such that growth is significantly inhibited after austenite formation during subsequent normalizing heat treatment, thereby a size of the ferrite grains produced during cooling is finely controlled. This is to improve both hydrogen-induced cracking resistance (HIC resistance) and low-temperature impact toughness.

One of the major ideas of the present disclosure is to provide a microstructure maximally inclusive of a ferrite fraction and minimally inclusive of cementite having a disadvantageous microstructure, and a hard phase such as pearlite, martensite-austenite complex phase (MA), or the like such that HIC propagation resistance and strength are simultaneously secured. To this end, hot rolling (controlled rolling) and water cooling (controlled cooling) are performed to produce nano-sized fine precipitates are produced in ferrite grains such that growth is significantly inhibited after austenite formation during subsequent normalizing heat treatment, thereby a size of the ferrite grains produced during cooling is finely controlled. This is to improve both hydrogen-induced cracking resistance (HIC resistance) and low-temperature impact toughness.

To produce a high-strength normalizing steel material having excellent HIC resistance and low-temperature impact toughness, the present disclosure controls a content of C to 0.12 wt% or less, a lower ranged as compared to a conventional method, controls the microstructure to contain 90% or more of the ferrite. Further, the present disclosure controls cooling conditions after hot rolling, such that the ferrite has 0.03 wt% or more of fine precipitates having a size of 100 nm or less in the ferrite grains such that growth is significantly inhibited after austenite formation, thereby having ferrite grains having an average grain size of 20 *µ*m or less produced during cooling, and at least one of pearlite, cementite, and martensite-austenite complex phase MA having a fraction of 10% by area or less. In addition, large amount of fine precipitates provide not only increasing strength but also site for absorbed hydrogen. Therefore, the present disclosure provides a high-strength steel material having excellent hydrogen-induced cracking resistance (HIC resistance) and low-temperature impact toughness and a manufacturing method therefore.

Hereinafter, the high-strength steel material having excellent HIC resistance and low-temperature impact toughness according to a preferable aspect is described in detail.

The high-strength steel material having excellent HIC resistance and low-temperature impact toughness according to a preferable aspect contains, by weight%, 0.02% to 0.12% of C, 0.02% to 0.60% of Si, 0.6 to 1.6% of Mn, 0.020% or less of P (excluding 0%), 0.003% or less of S (excluding 0%), 0.002% to 0.060% of sol.Al, 0.005% to 0.6% of Cu, 0.005% to 1.0% of Ni, 0.005% to 0.5% of Cr, 0.01% to 0.3% of Mo, 0.001% to 0.10% of Ti, 0.001% to 0.06% of Nb, 0.001% to 0.10% of V, 0.001% to 0.006% of N, 0.0002% to 0.0060% of Ca, a remainder of Fe and inevitable impurities, with (Ti+V+0.5Nb+0.5Mo) being 0.05% or greater and (Ti+V+0.5Nb+0.5Mo)/C being 0.8 or greater, the steel material having a microstructure inclusive of ferrite; and at least one of pearlite, cementite, and martensite-austenite complex phase (MA), wherein the ferrite has a fraction of 90% by area or more (excluding 100%), and wherein the ferrite includes 0.03 wt% or more of fine carbonitride precipitates having an average size of 100 nm or less and is 20 µm or less in average grain size.

Hereinafter, ingredients and scopes thereof are described.

### C: 0.02 wt% to 0.12 wt% (hereinafter, "%")

In normalizing steel, carbon (C) is generally added to secure tensile strength by forming pearlite, cementite or an MA phase; however, in the present disclosure, C is also added as an important element for producing fine precipitates having a size of 100 nm or less, and is preferably added in an amount of 0.02% to 0.12%. When the content of C is less than 0.02%, fractions of the carbonitride precipitate and the pearlite are lowered, thereby reducing the tensile strength of a matrix. When the content of C exeeds 0.12%, an excessive amount of a hard phase, such as pearlite, is produced and is present in the form of a band in the subsequent rolling process, thereby reducing not only the low-temperature impact toughness but also the HIC resistance. A more preferable content of C is 0.03% to 0.10%, and even more preferable content of C is 0.05% to 0.08%.

### Si: 0.02% to 0.60%

Silicon (Si) is an element added for solid solution strengthening in addition to deoxidation and desulfurization effects. It is preferable that Si be added in an amount of 0. 02% or more to secure yield strength and tensile strength.

Meanwhile, when Si is added in an amount exceeding 0.60%, weldability and low-temperature impact toughness are reduced, and a surface of manufactured steel plate is easily to be oxidized, thereby excessively creating an oxide film for deoxidizing steel. In this regard, it is preferable that an amount of Si 0.02% to 0.60%, more preferably 0.05% to 0.45%, most preferably 0.05% to 0.35%.

### Mn: 0.6 to 1.6%

Manganese (Mn) is an element having a high strength increasing effect by solid solution strengthening and is preferably added in an amount of 0.6% or more. Meanwhile, when Mn is excessively added, severe segregation occurs in a center in a thickness direction of the steel plate as well as causing formation of MnS, a non-metal inclusion together with segregated S. The MnS inclusion created in the center is elongated by subsequent rolling and thus greatly reduces low-temperature impact toughness and HIC resistance. In this regard, the content of Mn is preferably 1.6% or less, more preferably 0.8% to 1.45%, most preferably 1.1% to 1.3%.

### P: 0.020% or less (excluding 0%)

Phosphorus (P) is an element effective in increasing strength when added but greatly deteriorating low temperature toughness due to grain boundary segregation, especially in heat treated steel. Accordingly, it is desirable that an amount of P be managed as low as possible. Meanwhile, it is too expensive to excessively remove P in a steel manufacture process, and thus, it is preferable that the amount of P be limited to 0.020% or less (excluding 0%).

### S: 0.003% or less (excluding 0%)

Sulfur (S) is a representative element, which is combinded with Mn to produce the MnS inclusion in the center of the steel plate in the thickness direction, thereby not only deteriorating low-temperature toughness but also causing HIC and propagation. Accordingly, to secure HIC resistance, S needs to be eliminated during the steel manufacture process as much as possible; however, this may be high-priced. Accordingly, it is preferable that a content of S be limited to 0.003% or less, more preferably 0.001% or less.

### Sol.Al: 0.002% to 0.060%

Aluminum (Al), in addition to Si and Mn, is added as a strong deoxidizing agent during the steel manufacture process, and the deoxidizing effect can be maximally obtained by adding the same in an amount of at least 0.002% when used alone or in complex deoxidation. Meanwhile, when added in an amount exceeding 0.060%, the effect is saturated, and a fraction of Al₂O₃, one of oxidative inclusions produced as a result of the deoxidation, increases more than necessary, resulting in a coarse size and uneasy removal during refining. Accordingly, the content of sol.Al is preferably 0.002% to 0.06%, more preferably 0.005% to 0.04%, most preferably 0.01% to 0.025%.

### Cu: 0.005% to 0.6%

Copper (Cu) is an ingredient added due to its effects of significantly increasing strength by solid solution and precipitation and inhibiting corrosion in a wet hydrogen sulfide atmosphere. An excessive Cu addition causes cracking on a surface of the steel plate. Besides, in view of economic efficiency, Cu, as an expensive element, is preferably added in an amount of 0.005% to 0.6%, more preferably 0.02% to 0.4%, most preferably 0.05% to 0.3%.

### Ni: 0.005% to 1.0%

Nickel (Ni), although barely having a strength-increasing effect, is effective in improving low-temperature toughness. In particular, in the case of adding Cu, Ni has an effect of suppressing surface cracking caused by selective oxidation, which may occur when reheating a slab. Ni is added to obtain such an effect. Ni is also an expensive element and is thus, in view of economic efficiency, preferably added in an amount of 0.005% to 1. 0%, more preferably 0.02% to 0.5%, most preferably 0.05% to 0.3%.

### Cr: 0.005% to 0.5%

Chromium (Cr) has an insignificant effect of increasing yield strength and tensile strength by solid solution, but is effective in slowing down a cementite decomposition rate during heat treatment after welding or tempering, thereby preventing decrease in strength. For this, it is preferable to add 0.005% or more of Cr. Meanwhile, when the content of Cr exceeds 0.5%, not only a manufacturing cost rises, but also weldability is deteriorated. Accordingly, it is preferable that the content of Cr is limited to 0.5% or less, more preferably 0.01% to 0.4%, most preferably 0.02% to 0.2%.

### Mo: 0.01% to 0.3%

Molybdenum (Mo), which is an element effective in preventing a decrease in strength during tempering or heat treatment after welding, has an effect of preventing deterioration of toughness from being deteriorated by grain boundary segregation of impurities such as P. Mo, in the present disclosure, produces nano-sized carbonitrides to be caused for strength improvement. To this end, Mo is added in an amount of 0.01% or more.

Meanwhile, Mo is an expensive element and excessively increases hardenability when added in an amount exceeding 0.3%, thereby causing a hard phase deteriorating toughness and HIC resistance. In this regard, it is preferable that the content of Mo be limited to 0.01% to 0.3%, more preferably 0.02% to 0.2%, most preferably 0.05% to 0.15%.

### Ti: 0.001∼0.10%

Titanium (Ti) is added in an amount of 0.001% or more due to its effect of significantly increasing nano-sized carbonitrides upon addition. When added in an amount exceeding 0.10%, however, Ti may result in coarse TiN shaped hexagonal precipitates, thereby HIC and disadvantageous results in an impact experiment at low temperatures. Accordingly, the content of Ti is preferably limited to 0.10% or less, more preferably 0.002% to 0.05%, most preferably 0.005% to 0.03%.

### Nb: 0.001% to 0.06%

Niobium (Nb) is dissolved in austenite when reheating a slab, thereby increasing hardenability of austenite and is precipitated as carbonitrides, aligned with the matrix at high temperatures, upon hot rolling, thereby suppressing recrystallization during rolling or cooling to allow a final microstructure to be finely formed. Further, fine precipitates having a size of 100 nm or less are produced during transformation after cooling, thereby greatly increasing strength.

Meanwhile, when Nb is excessively added, coarse precipitates are likely to be formed in the center in the thickness direction, and hardenability of a weld zone is increased more than necessary, thereby deteriorating low-temperature toughness and HIC resistance. In this regard, Nb is preferably added in an amount of 0.001% to 0.06%, more preferably 0.002% to 0.05%, most preferably 0.005% to 0.04%.

### V: 0.001% to 0.10%

Vanadium (V) has almost no reinforcement effect due to precipitation or solid solution in a rolling as almost all of the slab is dissolved again during reheating, but has an effect of improving strength by being precipitated as ultrafine carbonitrides during tempering or in post-welding heat treatment. Due to its high price, it is preferable that a content of V to 0.001% be limited to 0.001% to 0.10%, more preferably 0.001% to 0.06%, most preferably 0.005% to 0.02%.

### N: 0.001∼0.006%

Nitrogen (N) is an element which may form a precipitation along with added Nb, Ti, and Al and may refine grain of steel to improve strength and toughness of a base metal. However, an excessive amount of N may result in a residual atomic state, which may cause embrittlement at high temperatures. Further, a re-solid solution fraction of the carbonitrides is reduced during slab reheating, thereby decreasing a formation amount of fine precipitates, which are a significant means of the present disclosure. In this regard, a content of N, in consideration of those of Nb, V, Mo and Ti as well as a reheating temperature, is preferably 0.001% to 0.006%, more preferably 0.002% to 0.005%, most preferably 0.002% to 0.0045%.

### Ca: 0.0002% to 0.0060%

Calcium (Ca), when added after Al deoxidation, binds to S present in the form of MnS to suppress formation of MnS while forming CaS having a spherical shape, thereby exhibiting an effect of suppressing HIC. Accordingly, to sufficiently form the added S in the form of CaS, it is preferable that Ca be added in an amount of 0.0002% or more. Meanwhile, an excessive amount of Ca is added, residual Ca is combined with oxygen (O) to produce coarse oxidative inclusions, thereby causing elongation and fracture during subsequent rolling and thus causing HIC. In this regard, an upper limit of the Ca amount is preferably limited to 0.0060%. The Ca amount is more preferably 0.0005% to 0.0060%, most preferably 0.001 to 0.0025%.

### (Ti+V+0.5Nb+0.5Mo): 0.05% or greater, (Ti+V+0.5Nb+0.5Mo)/C: 0.8 or greater

A reason for limiting the contents of Ti, Nb, V and Mo, which are elements producing denitrified precipitates, by the above formula is to sufficiently produce nano-sized fine precipitates during normalizing heat treatment such that growth of austenite is suppressed, and ferrite grains are fined. In addition, strength significantly increases due to the fine precipitates. Accordingly, the contents thereof need to be at least a certain level.

In addition, a ratio of C, an important constituting element of the carbonitride, needs to be high such that the fine precipitates can be sufficiently produced.

In this regard, it is preferable that (Ti+V+0.5Nb+0.5Mo) and (Ti+V+0.5Nb+0.5Mo)/C be limited to 0.05% or greater and 0.8% or greater, respectively.

The high-strength steel material having excellent hydrogen-induced cracking resistance and low-temperature impact toughness according to a preferable aspect of the present disclosure has a microstructure inclusive of ferrite; and at least one of pearlite, cementite, and martensite-austenite complex phase (MA), wherein the ferrite has a fraction of 90% by area or more (excluding 100%), and wherein the ferrite includes 0.03 wt% or more of fine carbonitride precipitates having an average size of 100 nm or less and is 20 µm or less in average grain size.

The steel material contains 90% or more (excluding 100%) of ferrite; and the remaining 10% or less of at least one of pearlite, cementite and martensite-austenite complex phase MA.

The pearlite, cementite and martensite-austenite complex phase MA are significantly effective in improving strength of a steel plate, in particular tensile strength; however, excessive amounts thereof may enlarge or elongate by rolling. In this case, low-temperature impact toughness is deteriorated, and in particular, they act as generation and propagation of HIC, thereby rapidly deteriorating the HIC resistance. Accordingly, an entire fraction of at least one of the pearlite, cementite and MA is preferably limited to 10% by area or less.

The pearlite may be present in a finely dispersed form in which a degree of orientation (omega_12) defined by ASTM E1268 of 0.1 or less, instead of having a banded structure. Such finely dispersed pearlite is present between fine ferrite grains.

The steel material is manufactured by a manufacturing method of a steel material including normalizing heat treatment. Fractions of the ferrite, pearlite, cementite and MA in the microstructure after the normalizing heat treatment of the steel material are increased by 10% or more, reduced by 10% or less, increased by 5% or less, and reduced by 3% or less, respectively.

Fine carbonitride precipitates having an average size of 100 nm or less are present in the ferrite in an amount of 0.03% wt or more.

When the fine carbonitride precipitates are contained in an amount of less than 0.03 wt%, the austenite growth cannot be suppressed during the normalizing heat treatment, leading to production of coarse austenite and production of coarse pearlite during subsequent cooling. In addition, there is a risk of significantly reduced effects of increased strength and fixed hydrogen by the precipitates.

An average grain size of the ferrite is 20 µm or less.

When the average grain size of the ferrite is exceeding 20 µm, strength by refining microstructure and HIC resistance may be reduced.

The steel material may have tensile strength of 485 MPa or greater, impact absorbed energy at -40°C of 120 J or greater, and a crack length ratio (CLR) of 5% or less in hydrophobic interaction chromatography (HIC) test.

The steel material may have a thickness of 6 mm to 133 mm.

Hereinafter, a method for manufacturing a high-strength steel material having excellent hydrogen-induced cracking resistance (HIC resistance) and low-temperature impact toughness according to another preferable aspect is described.

The method for manufacturing a high-strength steel material having excellent hydrogen-induced cracking resistance (HIC resistance) and low-temperature impact toughness according to another preferable aspect includes reheating a slab comprising by weight%, 0.02% to 0.12% of carbon (C), 0.02% to 0.60% of silicon (Si), 0.6 to 1.6% of manganese (Mn), 0.02% or less of phosphorus (P) (excluding 0%), 0.003% or less of sulfur (S) (excluding 0%), 0.002% to 0.060% of sol. aluminum (sol.Al), 0. 005% to 0.6% of copper (Cu), 0. 005% to 1. 0% of nickel (Ni), 0.005% to 0.5% of chromium (Cr), 0.01% to 0.3% of molybdenum (Mo), 0.001% to 0.10% of titanium (Ti), 0.001% to 0.06% of niobium (Nb), 0.001% to 0.10% of vanadium (V), 0.001% to 0.006% of nitrogen (N), 0.0002% to 0.0060% of calcium (Ca), a remainder of iron (Fe) and inevitable impurities, with (Ti+V+0.5Nb+0.5Mo) being 0.05% or greater and (Ti+V+0.5Nb+0.5Mo)/C being 0.8 or greater to 1080°C to 1300°C; hot rolling the reheated slab to a finish hot rolling temperature of 850°C or higher to obtain a hot rolled steel plate; water cooling the hot rolled steel plate to 550°C to 750°C; and performing normalizing heat treatment the cooled steel plate to 850°C to 950°C for 1.3*t [where t refers to thickness of steel plate (mm)] + (5 minutes to 60 minutes).

### Reheating

A slab having the above-described composition is reheated to 1080°C to 1300°C.

When the reheating temperature is less than 1080°C, it is difficult to dissolve carbides again, and the like, produced in the slab during continuous casting. When the reheating temperature exceeds 1300°C, coarse austenite grains are produced, thereby significantly deteriorating mechanical properties of the steel plate, such as tensile strength, low-temperature toughness, and the like. In particular, the reheating needs to be raised to a temperature, at which the added Ti, Nb, V, Mo, and the like are sufficiently dissolved. In this regard, the reheating temperature of the slab is preferably 1080°C to 1300°C, more preferably 1150°C to 1280°C.

### Obtaining hot rolled steel material

The slab reheated as the above is subject to controlled rolling in a condition, in which finish hot rolling temperature is 850°C or higher, to obtain a hot rolled steel material.

If the reheated slab is subject to general rolling, the hot rolling finishes at an extremely high temperature, leading to insignificant grain refining effect. Also, if the controlled rolling is performed at extremely low temperatures, re-dissolved Nb, and the like, are precipitated as a carbonitride. The precipitates produced at higher temperatures have a large size and thus significantly reduce suppression of austenite grain growth during subsequent normalizing process. Further, coarse composite inclusions produced in a refining process need to accept a deformation by rolling as strength of the steel plate increases upon decrease of the rolling temperature, whereby the inclusions are segmented into small size inclusions, or amorphous inclusions are elongated. The elongated or segmented inclusions are a factor directly related to the HIC occurrence and propagation. In consideration of the above, the finish hot rolling temperature is preferably limited to 850°C or higher, more preferably 850°C to 1050°C. The finish hot rolling temperature may be Ar₃ + 70°C to Ar₃ + 270°C.

The hot rolled steel material may have a thickness of 6 mm to 133 mm.

### Controlled cooling

The hot rolled steel material is water cooled to 550°C to 750°C and then air-cooled.

The steel material controlled rolled as the above is then subject to controlled cooling involving water cooling and air cooling. Performing water cooling after the controlled rolling can mostly prevent production of ferrite at high temperatures during the water cooling and serves to produce ferrite at a comparatively low temperature as compared to air cooling, resulting in a great refinement effect. In particular, when the cooling is performed in a temperature range of 550°C to 750°C, fine carbonitrides as well as ferrite are produced. The precipitates produced at this time are fine, 100 nm or less. When the cooling temperature exceeding 750°C, the ferrite is produced at higher temperatures and become coarse, and the precipitate are produced to be coarse, thereby significantly reducing the effect. Meanwhile, when the cooling temperature is less than 550°C, fine precipitates are not produced, thereby reducing to secure sufficient strength. In the case of a high cooling speed, ferrite production is suppressed, and hard phase such as bainite is produced, thereby increasing strength but reducing toughness at lower temperatures. Accordingly, the cooling temperature of the controlled cooling is preferably limited to 550°C to 750°C, more preferably 580°C to 670°C, in consideration of ingredients, rolling conditions, and the like.

The post controlled cooling steel material may contain 90% or more of the ferrite (excluding 100%), 10% or less of an entire fraction of at least one of pearlite, cementite and MA, while containing 0.03 wt% of the fine precipitates having an average size of 100 nm in the ferrite.

### Normalizing heat treatment

The steel material cooled as the above are allowed to maintain at 850°C to 950°C for 1.3*t [where t refers to thickness of steel plate (mm)] + (5 minutes to 60 minutes), and is subject to normalizing heat treatment involving air cooling.

When a normalizing heat treatment temperature is less than 850°C, it is difficult to secure strength of the steel plate as it is difficult to dissolve solute atoms for solid solution again. Meanwhile, when the normalizing heat treatment is performed at a temperature exceeding 950°C, low-temperature toughness is deteriorated as crystal grains grow.

A reason for limiting a maintaining time during the normalizing heat treatment is that homogenization of a structure becomes difficult if the maintaining time is shorter than a reference time, and productivity is impaired if the maintaining is longer.

Accordingly, it is preferable that the normalizing heat treatment be maintained for 1.3*t [where t refers to thickness of steel plate (mm)] + (5 minutes to 60 minutes).

The microstructure of steel material microstructure after the normalizing heat treatment may include ferrite; and at least one of pearlite, cementite, and martensite-austenite complex phase (MA), wherein the ferrite has a fraction of 90% by area or more (excluding 100%), and wherein the ferrite includes 0.03 wt% or more of fine carbonitride precipitates having an average size of 100 nm or less and is 20 µm or less in average grain size.

As for the fractions of the ferrite, pearlite, cementite and MA in the steel material microstructure after the normalizing heat treatment, as compared to those before the normalizing heat treatment, a fraction of the ferrite may be increased by 10% or less and that of the pearlite may be reduced by 10% or less, while that of the cementite may be increased by 5% or less and that of the MA may be reduced by 3% or less.

As previously described, by optimally controlling a steel composition, controlled rolling, controlled cooling and normalizing heat treatment according to the present disclosure, a high-strength steel material having excellent low-temperature toughness and HIC resistance can be effectively manufactured by fining the structure as well as minimizing the hardened structure of the pearlite, cementite, MA, and the like, which are disadvantageous in terms of toughness and HIC resistance, as compared to a conventional method.

### Tempering heat treatment

The normalizing heat treated steel material may be subject to tempering heat treatment at 500°C or higher for 10 minutes or more.

The tempering heat treatment may be performed to improve toughness and strength at lower temperatures. A tempering temperature is preferably performed at 500°C or higher. When the tempering temperature is less than 500°C, remaining stress of the steel material is not smoothly removed, or desired fine precipitates are not significantly produced. When the tempering heat treatment is performed for less than 10 min, the production of precipitates is reduced, and thus is preferably performed for 10 minutes or more.

The tempering heat treatment may serve to increase the fraction of the ferrite in the microstructure of the steel material by 3% or less by area and decrease the entire fraction of the pearlite, cementite and MA by 3% by area.

Due to tempering heat treatment, an amount of the carbonitride precipitate in the steel material may be increased by 0.001 wt% to 0.005 wt%.

### [Mode for Invention]

Hereinafter, the present disclosure is described in more detail with reference to the following example embodiments.

A slab having a steel composition (chemical composition) of Table 1 below is reheated under manufacturing conditions indicated in Table 2 below, and the reheated slab was then subject to controlled rolling to obtain a hot rolled steel material having a thickness of Table 2, followed by controlled cooling and normalizing heat treatment, thereby manufacturing a steel material.

The normalizing heat treatment was performed for 1.3*t [where t refers to thickness of steel plate (mm)] + 20 min.

Inventive Materials (a to c) in Table 1 below are consistent with the steel composition of the present disclosure, and Comparative Materials (d to h) are outside of the steel composition of the present disclosure.

The steel material manufactured as described above was measured with respect to a ferrite fraction (area%), an average grain size (µm), an amount of fine precipitates (wt%), an average size of fine precipitates (nm), a pearlite fraction (area%), and yield strength (MPa), tensile strength (MPa), impact absorbed energy (J, -45°C) and HIC CLR (%) after normalizing heat treatment are investigated, and a result thereof is shown in Tables 3 and 4 below.

In Table 3 below, the structure of the microstructure, excluding ferrite and pearlite, is at least one of cementite and MA.

Meanwhile, as for Inventive Example 1 and Comparative Example 3, the microstructures and precipitate distributions were observed, and results thereof are shown in FIGS. 1 to 4. FIG. 1 is a photograph of a microstructure of Comparative Example 3, and FIG. 2 is a photograph of a microstructure of Inventive Example 1 while FIG. 3 is a photograph of a precipitate distribution of Comparative Example 3, and FIG. 4 is a photograph of a precipitate distribution of Inventive Example 1.

**[Table 1]**

| Classification | | Chemical Composition (wt%) | | | | | | | | | | | | | | | | |
|---|---|---|---|---|---|---|---|---|---|---|---|---|---|---|---|---|---|---|
| | | C | Si | Mn | P | s | Sol.Al | Cu | Ni | Cr | Mo | Ti | Nb | V | N | Ca | Ti+V+0.5Nb+0.5Mo | (Ti+V+0.5Nb+0.5Mo)/C |
| Invent ive material | a | 0.055 | 0.32 | 1.14 | 0.003 | 0.0005 | 0.027 | 0.23 | 0.15 | 0.06 | 0.08 | 0.023 | 0.008 | 0.009 | 0.0032 | 0.0016 | 0.07 6 | 1.38 |
| | b | 0.035 | 0.22 | 1.45 | 0.003 | 0.0008 | 0.031 | 0.01 | 0.14 | 0.02 | 0.12 | 0.043 | 0.002 | 0.002 | 0.0041 | 0.0012 | 0.106 | 3.03 |
| | c | 0.081 | 0.43 | 0.91 | 0.005 | 0.0004 | 0.015 | 0.01 | 0.01 | 0.12 | 0.03 | 0.083 | 0.021 | 0.012 | 0.0029 | 0.0013 | 0.121 | 1.49 |
| Comparative material | d | 0.041 | 0.32 | 1.45 | 0.007 | 0.001 | 0.032 | 0.01 | 0.02 | 0.04 | 0.05 | 0.011 | 0.0 02 | 0.0 03 | 0.0042 | 0.0013 | 0.040 | 0.98 |
| | e | 0.145 | 0.38 | 1.35 | 0.007 | 0.0009 | 0.022 | 0.12 | 0.33 | 0.02 | 0.11 | 0.012 | 0.0 03 | 0.002 | 0.0032 | 0.0021 | 0.071 | 0.49 |
| | | | | | | | | | | | | | | | | | | |
| | f | 0.089 | 0.33 | 0.82 | 0.006 | 0.0008 | 0.035 | 0.02 | 0.01 | 0.02 | 0.42 | 0.001 | 0.0 03 | 0.002 | 0.0045 | 0.0012 | 0.215 | 2.41 |
| | g | 0.102 | 0.15 | 1.08 | 0.005 | 0.001 | 0.021 | 0.11 | 0.02 | 0.03 | 0.05 | 0.15 | 0.0 05 | 0.006 | 0.0034 | 0.0023 | 0.184 | 1.80 |
| | h | 0.061 | 0.31 | 1.25 | 0.008 | 0.0009 | 0.035 | 0.01 | 0.03 | 0.02 | 0.09 | 0.021 | 0.0 03 | 0.003 | 0.0088 | 0.0018 | 0.071 | 1.16 |

**[Table 2]**

| | Classification | Thickness (mm) | Temperature of slab reheating (°C) | Temperature of finish hot rolling (°C) | Temperature of cooling (°C) | Temperature of normalizing (°C) |
|---|---|---|---|---|---|---|
| Inventive Ex 1 | a | 30.0 | 1230 | 880 | 635 | 891 |
| Inventive Ex 2 | b | 9.5 | 1190 | 862 | 712 | 903 |
| Inventive Ex 3 | c | 95.0 | 1163 | 982 | 623 | 888 |
| Comparative Ex 1 | b | 25.0 | 1062 | 885 | 642 | 916 |
| Comparative Ex 2 | c | 45.0 | 1163 | 936 | 513 | 913 |
| Comparative Ex 3 | c | 80.0 | 1134 | 981 | - | 905 |
| Comparative Ex 4 | d | 51.0 | 1223 | 963 | 635 | 899 |
| Comparative Ex 5 | e | 30.0 | 1198 | 924 | 621 | 913 |
| Comparative Ex 6 | f | 12.0 | 1178 | 872 | 602 | 900 |
| Comparative Ex 7 | g | 78.0 | 1192 | 974 | 655 | 897 |
| Comparative Ex 8 | h | 25.0 | 1153 | 875 | 638 | 887 |

**[Table 3]**

| | Classification | Thickness (mm) | Ferrite fraction (%) | Amount of fine precipitate (%) | Pearlite fraction (%) | Degree of orientation of pearlite (omega_12) | Ave grain diameter of ferrite (µm) | Ave diameter of precipitate (nm) |
|---|---|---|---|---|---|---|---|---|
| Inventive Ex 1 | a | 30.0 | 96.2 | 0.046 | 2.2 | 0.04 | 17 | 35 |
| Inventive Ex 2 | b | 9.5 | 98.9 | 0.065 | 0.7 | 0.04 | 13 | 48 |
| Inventive Ex 3 | c | 95.0 | 92.1 | 0.074 | 4.6 | 0.07 | 15 | 41 |
| Comparative Ex 1 | b | 25.0 | 98.9 | 0.022 | 0.9 | 0.02 | 23 | 55 |
| Comparative Ex 2 | c | 45.0 | 92.1 | 0.024 | 4.6 | 0.07 | 22 | 37 |
| Comparative Ex 3 | c | 80.0 | 88.2 | 0.015 | 8.5 | 0.07 | 31 | 120 |
| Comparative Ex 4 | d | 51.0 | 98.4 | 0.024 | 1.0 | 0.02 | 16 | 45 |
| Comparative Ex 5 | e | 30.0 | 83.7 | 0.043 | 9.6 | 0.17 | 25 | 113 |
| Comparative Ex 6 | f | 12.0 | 89.9 | 0.131 | 3.7 | 0.11 | 17 | 63 |
| Comparative Ex 7 | g | 78.0 | 88.2 | 0.112 | 6.9 | 0.12 | 26 | 145 |
| Comparative Ex 8 | h | 25.0 | 95.4 | 0.009 | 2.7 | 0.05 | 23 | 36 |

**[Table 4]**

| | Classification | Post-normalizing yield strength (MPa) | Post-normalizing tensile strength (MPa) | Post-normalizing impact absorbed energy (J, -49°C) | Post-normalizing HIC CLR (%) |
|---|---|---|---|---|---|
| Inventive Ex 1 | a | 348 | 501 | 253 | 0.0 |
| Inventive Ex 2 | b | 380 | 515 | 314 | 0.0 |
| Inventive Ex 3 | c | 314 | 500 | 157 | 0.0 |
| Comparative Ex 1 | b | 319 | 447 | 301 | 0.0 |
| Comparative Ex 2 | c | 305 | 458 | 198 | 0.0 |
| Comparative Ex 3 | c | 281 | 412 | 67 | 52.0 |
| Comparative Ex 4 | d | 321 | 446 | 272 | 0.0 |
| Comparative Ex 5 | e | 354 | 522 | 49 | 12.0 |
| Comparative Ex 6 | f | 365 | 592 | 34 | 23.0 |
| Comparative Ex 7 | g | 337 | 517 | 61 | 7.0 |
| Comparative Ex 8 | h | 344 | 455 | 275 | 0.0 |

As shown in Tables 3 and 4, the steel materials (Inventive Examples 1 to 3) manufactured according to the steel composition and manufacturing conditions of the present disclosure has tensile strength of 485 MPa or more, impact absorbed energy at -40°C of 120 J or greater, and CLR of 5% or less in HIC test. Such a steel material of the present disclosure is significantly effective to be used as a steel material for maritime structures and pressure vessels.

Meanwhile, the ingredients of Comparative Example 1 fall within the scope of the present disclosure; however, a slab reheating temperature is lower than the temperature range of the present disclosure, thus making the coarse carbonitride precipitates produced during slab manufacturing difficult to be dissolved again. Accordingly, a fraction of the fine precipitates produced during rolling and cooling is significantly reduced, resulting in almost no increase in the strength improving effect after normalizing.

Comparative Example 2 is the case in which the ingredients fall within the scope of the present disclosure; however, a cooling temperature after rolling is below the temperature range of the present disclosure, thereby giving rise to a reduced speed of precipitate production and insufficient production of carbonitrides. In this case, the post-normalizing strength is not sufficiently secured.

Comparative Example 3 is a case in which the ingredients fall within the scope of the present disclosure; however, controlled cooling is not applied after rolling and air-cooling as conventional manufacturing method is involved. Due to a significantly low cooling speed, ferrite is transformed at high temperatures, thereby producing coarse ferrite. In addition, fine precipitates are insufficiently produced. In this case, a final microstructure, as shown in FIG. 1, has not only coarse ferrite (white-colored in the photo) but also pearlite including some M-A structures (black-colored in the photo) in the form of a band, thereby leading to insufficient strength and impact toughness as well as HIC characteristics.

Comparative Example 4 is the case in which added elements producing carbonitride are insufficient. Even when all manufacturing conditions fall within the scope of the present disclosure, an amount of the produced fine precipitates is insufficient, thus giving rise to insufficient strength secured.

Comparative Example 5 is the case in which an amount of C addition exceeds the scope of the present disclosure. The more C is contained, the more carbonitrides are precipitated; however, when a ratio of C is significantly higher than that of an alloy element, the coarse carbonitrides are produced. This may result in reduced suppression of austenite growth during subsequent normalizing, and the strength improvement effect is significantly reduced, thereby deteriorating both strength and low-temperature toughness.

Comparative Example 6 is the case in which an amount of Mo addition exceeds the scope of the present disclosure. Mo is an important element for producing fine precipitates while greatly improving hardenability of a steel material such that remaining austenite is formed as a MA constituent during cooling after normalizing.

Comparative Example 7 is the case in which an amount of Ti addition exceeds the scope of the present disclosure. Ti is the most important element for producing fine precipitates; however, coarse precipitates are produced when an excessive amount thereof is added. This causes destruction, ultimately resulting in significantly deteriorated low-temperature toughness and HIC resistance.

Comparative Example 8 is the case in which an amount of N addition exceeds the scope of the present disclosure. When an excessive amount of N is added, a re-solid solution amount of the coarse carbonitride, produced during slab manufacturing, is significantly reduced even when a reheating temperature increases. Accordingly, even when subsequent manufacturing conditions fall within the scope of the present disclosure, a fraction of the produced fine carbonitrides greatly decrease, thereby failing to obtain sufficient strengthening effect.

Meanwhile, the steel material (Comparative Example 3) manufactured according to a conventional method has pearlite having a banded structure as illustrated in FIG. 1, whereas that the steel material (Inventive Example 1) manufactured according to the present disclosure has pearlite finely dispersed instead of having the banded structure as illustrated in FIG. 2. Besides, the steel material (Inventive Example 1) manufactured according to the present disclosure (FIG. 4), as compared to that the steel material (Comparative Example 3) manufactured according to a conventional method (FIG. 3), contains more fine precipitates dispersed.

As previously described, in the case of manufacturing a steel material according to the steel composition and manufacturing conditions of the present disclosure, effects of high strength, excellent low-temperature toughness and HIC resistance can be obtained through structure refinement while minimizing a hardened structure of pearlite, or the like, which is disadvantageous in toughness and HIC resistance, as compared to manufacturing a steel material according to a conventional method.

## Claims

1. A high-strength steel material having excellent hydrogen-induced cracking resistance and low-temperature impact toughness, comprising:
by weight%, 0.02% to 0.12% of carbon (C), 0.02% to 0.60% of silicon (Si), 0.6 to 1.6% of manganese (Mn), 0.020% or less of phosphorus (P) (excluding 0%), 0.003% or less of sulfur (S) (excluding 0), 0.002% to 0.060% of sol. aluminum (sol.Al), 0.005% to 0.6% of copper (Cu), 0.005% to 1.0% of nickel (Ni), 0.005% to 0.5% of chromium (Cr), 0.01% to 0.3% of molybdenum (Mo), 0.001% to 0.10% of titanium (Ti), 0.001% to 0.06% of niobium (Nb), 0.001% to 0.10% of vanadium (V), 0.001% to 0.006% of nitrogen (N), 0.0002% to 0.0060% of calcium (Ca), a remainder of iron (Fe) and inevitable impurities, with (Ti+V+0.5Nb+0.5Mo) being 0.05% or greater and (Ti+V+0.5Nb+0.5Mo)/C being 0.8 or greater,
the steel material having a microstructure inclusive of ferrite; and at least one of pearlite, cementite, and martensite-austenite complex phase (MA), wherein the ferrite has a fraction of 90% by area or more (excluding 100%), and at least one of pearlite, cementite, and martensite-austenite complex phase MA has a fraction of 10% by area or less, and wherein the ferrite includes 0.03 wt% or more of fine carbonitride precipitates having an average size of 100 nm or less and is 20 µm or less in average grain size.

2. The high-strength steel material having excellent hydrogen-induced cracking resistance and low-temperature impact toughness of claim 1, wherein the pearlite is a finely distributed form in which the degree of orientation (omega_12) defined in ASTM E1268 of 0.1 or less.

3. The high-strength steel material having excellent hydrogen-induced cracking resistance and low-temperature impact toughness of claim 1, wherein the steel material has tensile strength of 485 MPa or greater, impact absorbed energy at -40°C of 120J or greater, and a crack length ratio (CLR) of 5% or less in hydrogen-induced cracking (HIC) test.

4. The high-strength steel material having excellent hydrogen-induced cracking resistance and low-temperature impact toughness of claim 1, wherein the steel material has a thickness of 6 mm to 133 mm.

5. A method for manufacturing a high-strength steel material having excellent hydrogen-induced cracking resistance and low-temperature impact toughness, comprising:
reheating a slab comprising by weight%, 0.02% to 0.12% of carbon (C), 0.02% to 0.60% of silicon (Si), 0.6 to 1.6% of manganese (Mn), 0.020% or less of phosphorus (P) (excluding 0%), 0.003% or less of sulfur (S) (excluding 0%), 0.002% to 0.060% of sol. aluminum (Sol.Al), 0.005% to 0.6% of copper (Cu), 0.005% to 1.0% of nickel (Ni), 0.005% to 0.5% of chromium (Cr), 0.01% to 0.3% of molybdenum (Mo), 0.001% to 0.10% of titanium (Ti), 0.001% to 0.06% of niobium (Nb), 0.001% to 0.10% of vanadium (V), 0.001% to 0.006% of nitrogen (N), 0.0002% to 0.0060% of calcium (Ca), a remainder of iron (Fe) and inevitable impurities, with (Ti+V+0.5Nb+0.5Mo) being 0.05% or greater and (Ti+V+0.5Nb+0.5Mo)/C being 0.8 or greater to 1080°C to 1300°C;
hot rolling the reheated slab to a finish hot rolling temperature of 850°C or higher to obtain a hot rolled steel plate;
water cooling the hot rolled steel plate to 550°C to 750°C; and
performing normalizing heat treatment the cooled steel plate to 850°C to 950°C for 1.3*t [where t refers to thickness of steel plate (mm)] + (5 minutes to 60 minutes).

6. The method for manufacturing a high-strength steel material having excellent hydrogen-induced cracking resistance and low-temperature impact toughness of claim 5, wherein in the step of reheating the slab, a reheating temperature is 1150°C to 1300°C.

7. The method for manufacturing a high-strength steel material having excellent hydrogen-induced cracking resistance and low-temperature impact toughness of claim 5, wherein the finish hot rolling temperature is 850°C to 1050°C.

8. The method for manufacturing a high-strength steel material having excellent hydrogen-induced cracking resistance and low-temperature impact toughness of claim 5, wherein the finish hot rolling temperature is Ar₃ + 70°C to Ar₃ + 270°C.

9. The method for manufacturing a high-strength steel material having excellent hydrogen-induced cracking resistance and low-temperature impact toughness of claim 5, wherein the hot rolled steel plate has a thickness of 6 mm to 133 mm.

10. The method for manufacturing a high-strength steel material having excellent hydrogen-induced cracking resistance and low-temperature impact toughness of claim 5, further comprising performing tempering heat treatment the normalizing heat treated steel plate to 500°C or higher for 10 minutes or more.

11. The method for manufacturing a high-strength steel material having excellent hydrogen-induced cracking resistance and low-temperature impact toughness of claim 10, wherein by the tempering heat treatment, a content of carbonitride precipitate in the steel plate is increased by 0.001 wt% to 0.005 wt%.
